

## UNITED STATES PATENT OFFICE

2,675,314

## ANTISTAIN AGENTS FOR PHOTOGRAPHIC COLOR MATERIALS

Paul W. Vittum, Arnold Weissberger, and John R. Thrtle, Rochester, N. Y., assignors to Eastman Kodak Company, Rochester, N. Y., a corporation of New Jersey

No Drawing. Application April 10, 1951,  
Serial No. 220,336

9 Claims. (Cl. 95—6)

1

This invention relates to color photography and particularly to the prevention of color staining or fog in photographic emulsions containing color couplers.

The incorporation of color-forming components or couplers in silver halide emulsion layers is well known. These couplers are compounds such as phenolic hydroxyl compounds or compounds with reactive methylene groups which are capable of reacting with the oxidation products of primary aromatic amino developing agents to produce indoaniline or azomethine dyes. The color couplers may be added directly to the emulsion layers as described in Fischer U. S. Patent 1,102,028, granted June 30, 1914 or they may be incorporated in a separate medium which is insoluble in the carrier for the sensitive silver halide as described in the Mannes and Godowsky U. S. Patent 2,304,940, granted December 15, 1942 and Jelley and Vittum, U. S. Patent 2,322,027, granted June 15, 1943.

In these processes in which the color couplers are incorporated in the emulsion layers, the addition of effective anti-stain agents to the emulsion layers has been found to confer instability to light upon some of the dye images formed in the emulsion layers. Hydroquinone derivatives and other reducing agents such as ascorbic acid have been used for this purpose. Because of the instability conferred upon the dye images, it has been found desirable to omit the anti-stain agent from the emulsion and this necessitates the use of an anti-stain agent in the processing solutions. Most of the compounds available for this purpose, however, have interfered with color development by decreasing the amount of dye formed or have yielded developer solutions which are unstable.

It is, therefore, an object of the present invention to provide novel and useful anti-stain agents for incorporation in silver halide emulsions containing color couplers. A further object is to provide suitable anti-stain agents for use in solutions used to process such emulsions. A still further object is to provide anti-stain agents which may be incorporated in photographic developer solutions for developing emulsions containing color couplers and which do not reduce the stability of such solutions. Other objects will appear from the following description of our invention.

These objects are accomplished by conducting the development of a silver halide emulsion containing one or more color couplers, with a primary

5

10

20

25

30

35

40

45

50

2

aromatic amino developing agent in the presence of a compound having the formula



in which A is hydrogen, an alkyl group, —NH<sub>2</sub>, —NHR, —NR<sub>2</sub>, or —OR;

R is an alkyl group such as methyl, ethyl, lauryl, hexadecyl, etc., or a substituted alkyl group such as hydroxyethyl, which may contain from 1 to 16 or more carbon atoms depending upon the use to which the anti-stain agent is placed;

B is =NOH or =O; and

n is 1 or 2.

Where we refer in the claims to an alkyl group, it is to be understood that we intend to include substituted alkyl groups.

The following examples illustrate the general class of compounds which we may use.



55



Compounds 1, 2, 4, 5, 6, 9, 10, 12 and 14 are designed for use as anti-stain agents to be applied during processing, that is, for treating the emulsion at any stage not later than development. They may be incorporated in the developing solution itself or in a pre-bath. Compounds 3, 7, 8, 11, 13 and 15 are suitable for incorporation in the emulsion layer during manufacture. In either case, the anti-stain agent will be present in the emulsion layer during color-forming development and it is essential that the development of the emulsion layer with the color developing agent takes place in the presence of the anti-stain agent. When the anti-stain agent is incorporated in the developer or in a pre-bath, it diffuses into the emulsion layer and is present in the emulsion layer at the time of development of the colored image.

The following example illustrates a developer solution useful for processing a multi-layer material containing color couplers.

*Example 1*

|                                             |       |    |      |
|---------------------------------------------|-------|----|------|
| 2-amino-5-diethylaminotoluene hydrochloride | ----- | g  | 3    |
| Sodium sulfite (anhyd.)                     | ----- | g  | 4    |
| Sodium carbonate (anhyd.)                   | ----- | g  | 20   |
| Potassium bromide                           | ----- | g  | 1    |
| Gentisaldoxime                              | ----- | g  | 0.5  |
| 6-nitrobenzimidazole nitrate                | ----- | g  | 0.03 |
| Water                                       | ----- | cc | 1000 |

The following example illustrates a pre-bath which may be used for two minutes immediately preceding color forming development to secure the advantages of our invention.

*Example 2*

|                         |       |    |      |
|-------------------------|-------|----|------|
| Sodium sulfite (anhyd.) | ----- | g  | 5    |
| Potassium bromide       | ----- | g  | 5    |
| Gentisamide             | ----- | g  | 1    |
| Water                   | ----- | cc | 1000 |

The following example illustrates the incorporation of the anti-stain agent in an emulsion layer.

*Example 3*

One gram of the coupler N-[4-(benzoylacetyl)amino]-benzene-sulfonyl]-N-(γ-phenylpropyl)-p-toluidine and 0.1 gram of the anti-stain agent N-(n-hexadecyl)-gentisamide were dissolved at 130° C. in 3 cc. of di-n-butylphthalate. This hot solution was poured with stirring into a solution containing 18 cc. of 10% gelatin, 2 cc. of water, and 2 cc. of 10% Alkanol B (sodium triisopropylnaphthalene sulfonate). The whole mixture was then passed several times through a colloid mill and the resulting fine dispersion was added, at 40° C. to 50 cc. of a melted posi-

5

tive-type emulsion. The mixture was then coated on a support in the normal manner and dried. The resulting coating gave a bright yellow dye image on color development and showed a marked reduction in stain over a similar material prepared without the anti-stain agent.

The compounds listed above were prepared as follows:

Compound 1 was prepared according to J. A. C. S., 63, 183 (1941).

Compound 2 was prepared according to J. Chem. Soc., 67, 998 (1895).

Compound 3 — 2,5-dihydroxylaurophenone (lauroylhydroquinone) was prepared according to J. Chem. Soc., 2112 (1931). Compound 3 can be made by the usual reaction with hydroxyl-amine:



Compound 4 was prepared as follows J. A. C. S., 63, 183 (1941):



Compound 5 can be prepared by the reaction of methyl gentisate (compound 10) with methylamine:



Compound 6 was prepared according to U. S. Patent 2,463,462 (1949).

Compound 7 can be synthesized as follows:



Compound 8 was prepared as follows:



Compound 9 can be prepared by the reaction of methyl gentisate with dimethylamine:



Compound 10 was prepared according to Ann., 340, 214 (1905).

Compound 11 was prepared as follows:



Compound 12 can be prepared as follows:



Compound 13 can be prepared like compound 12 by using dodecyl alcohol for the esterification.



Compound 14 can be prepared from compound 12 by reaction of the latter with ammonia.



Compound 15 can be prepared from compound 12 by reaction of the latter with n-hexadecylamine or by a series of reactions such as those described for compound 8.



Our method is intended for use principally with emulsions which produce a negative image upon direct development, that is, emulsions in which a negative image is formed upon development after exposure under a positive image or in which positive images are formed on development after exposure under a negative image. Our method may also be used with reversal color developers and with emulsions intended to be developed by reversal to form a colored image. Our agents are particularly useful with sensitive materials coated on paper supports, where it is especially important to reduce the minimum or fog densities. This applies both to negative-developed paper and to reversal paper and transparency materials.

It will be understood that the examples and modifications disclosed herein are by way of example only and that our invention is to be taken as limited only by the scope of the appended claims.

We claim:

1. In a process of color photography, the method of preventing color stain in a photographic silver halide emulsion having a non-diffusing color coupler therein, which comprises exposing said emulsion and developing it with a primary aromatic amino developing agent in the presence of a compound having the formula:



where A represents an alkyl radical.

2. In a process of color photography, the method of preventing color stain in a photographic silver halide emulsion having a non-diffusing color coupler therein, which comprises exposing said emulsion and developing it with a primary aromatic amino developing agent in the presence of a compound having the formula:



where A represents a trivalent amine radical.

3. In a process of color photography, the method of preventing color stain in a photographic silver halide emulsion having a non-diffusing color coupler therein, which comprises exposing said emulsion and developing it with a primary

aromatic amino developing agent in the presence of a compound having the formula:



where A represents an alkylamino group.

4. In a process of color photography, the method of preventing color stains on color images produced in a silver halide emulsion containing a color coupler, by development of said emulsion with a primary aromatic amino developing agent, and treating said emulsion at a stage not later than development, with a solution of a compound having the formula:



5. In a process of color photography, the method of preventing color stains on color images produced in a silver halide emulsion containing a color coupler, by development of said emulsion with a primary aromatic amino developing agent, and treating said emulsion at a stage not later than development, with a solution of a compound having the formula:

6. The method of preventing the formation of stain in a photographic silver halide emulsion having a non-diffusing color coupler compound therein, which comprises developing said emulsion after exposure, with a solution of a primary aromatic amino developing agent containing gentis-aldoxime.

6. The method of preventing the formation of stain in a photographic silver halide emulsion having a non-diffusing coupler compound therein, which comprises developing said emulsion after exposure, with a solution of a primary aromatic amino developing agent containing gentisamide.

7. The method of preventing the formation of stain in a photographic silver halide emulsion having a non-diffusing coupler compound therein, which comprises developing said emulsion after exposure, with a solution of a primary aromatic amino developing agent containing N-( $\beta$ -hydroxyethyl)-gentisamide.

8. A color-forming photographic silver halide emulsion having a non-diffusing color coupler incorporated therein, and containing 2,5-dihydroxyalauophenone oxime as an anti-stain agent.

9. A color-forming photographic silver halide emulsion having a non-diffusing color coupler incorporated therein, and containing N-n-hexadecylgentisamide as an anti-stain agent.

5 References Cited in the file of this patent

UNITED STATES PATENTS

| Number    | Name                | Date           |
|-----------|---------------------|----------------|
| 2,301,387 | Evans et al. -----  | Nov. 10, 1942  |
| 2,360,290 | Vittum et al. ----- | Oct. 10, 1944  |
| 2,384,658 | Vittum -----        | Sept. 11, 1945 |
| 2,403,721 | Jelley et al. ----- | July 9, 1946   |

15 FOREIGN PATENTS

| Number  | Country             | Date          |
|---------|---------------------|---------------|
| 501,040 | Great Britain ----- | May 10, 1937  |
| 545,732 | Great Britain ----- | June 10, 1942 |